

## UNITED STATES PATENT OFFICE

LEO KLÜGER, OF VIENNA, AUSTRIA, ASSIGNOR TO OESTERREICHISCHE SCHMIDT-STAHLWERKE A. G., OF VIENNA, AUSTRIA, AN AUSTRIAN COMPANY

## HIGH SPEED TOOL STEEL

No Drawing. Application filed November 11, 1932, Serial No. 406,536, and in Austria November 14, 1932.

So called self hardening steels for tools have already been proposed, some of which are tungsten manganese steels free from chromium while others are tungsten chromium steels, but it has never been proposed to use cobalt as a constituent in alloys of the above composition. Since in all self hardening steels the cutting capacity was comparatively small, steels containing cobalt and free from chromium and having a high cutting capacity had still less been proposed.

The known high speed tool steels on the other hand which since the beginning of this century have replaced on account of their high cutting capacity the self hardening steel previously used, have in all cases chromium for their main constituent and for another essential constituent tungsten or its equivalents and recently also cobalt has been frequently used for an additional constituent of such high speed tool steels. However, chromium is considered an essential constituent of all modern high speed tool steels having an adequate cutting capacity and is used in all cases. These known steels containing chromium and tungsten with or without the addition of cobalt offer difficulties in connection with practical use as regards their being worked in the heat, their being shaped in the cold and their thermic treatment.

Now it has been discovered that the cutting capacity of high speed tool steels containing cobalt without any addition of chromium is substantially the same as that of the chromium containing high speed tool steels heretofore used, but the working in the heat of such cobalt steels free from chromium, their shaping in the cold and their thermic treatment is much more easy and thus the difficulties above referred to met with in the case of chromium containing high speed tool steels are at least greatly reduced and to some extent even entirely removed.

The following figures give various examples of carrying my present invention into

effect. Especially the contents in the elements usually accompanying iron, such as manganese and silicon are given by way of examples only and are by no means limitative.

|          | C    | Mn    | Si   | W     | V    | Mo   | Co    | Ta   |
|----------|------|-------|------|-------|------|------|-------|------|
| (1)..... | 1.21 | 0.21  | 0.87 | 22.00 | 1.64 | 0.36 | 18.91 | 2.13 |
| (2)..... | 0.97 | 0.35  | 0.16 | 19.82 | 1.64 | 1.06 | 10.81 | 0.17 |
| (3)..... | 1.00 | 0.15  | 0.27 | 19.33 | 1.74 | 0.41 | 9.40  | 0.81 |
| (4)..... | 0.88 | 0.22  | 0.32 | 18.16 | 1.54 | 0.90 | 13.54 | 0.07 |
| (5)..... | 0.90 | Trace | 0.09 | 16.00 | 0.51 | 0.13 | 3.45  | 0.09 |

the balance being iron.

It will be seen that the contents in cobalt may vary within wide limits. Other constituents of the alloy such for instance as vanadium, molybdenum, tantalum, titanium, uranium and so on are either elements accompanying other constituents of the alloy or may be added in suitably higher proportions for special uses of the resulting alloy.

The advantages secured by the present invention are obtained to a smaller extent even in the presence of very small percentages of chromium, which may be simply considered as impurities.

The steels according to the present invention may be manufactured in various ways well known per se in the manufacture of high speed tool steels.

What I claim is:

1. A substantially chromium free high speed tool steel comprising in rough approximation:

Tungsten 16.5-22.50%

Cobalt 3.5-19.00%

Vanadium 0.5-1.75%

Carbon 0.9-1.25%

Tantalum 0.1-2.15%

Silicon 0.1-0.40%

Molybdenum 0.1-1.10%

Manganese up to 0.35%

and the remainder iron.

